

W. E. GREENAWALT.  
METALLURGICAL PROCESS.  
APPLICATION FILED NOV. 28, 1917.

1,344,127.

Patented June 22, 1920.



WITNESSEES

James Greenawalt  
Mars H. Wooldredge

INVENTOR  
William E. Greenawalt

# UNITED STATES PATENT OFFICE.

WILLIAM E. GREENAWALT, OF DENVER, COLORADO.

## METALLURGICAL PROCESS.

1,344,127.

Specification of Letters Patent. Patented June 22, 1920.

Application filed November 28, 1917. Serial No. 204,337.

To all whom it may concern:

Be it known that I, WILLIAM E. GREENAWALT, a citizen of the United States, residing in the city and county of Denver and State of Colorado, have invented certain new and useful Improvements in Metallurgical Processes, of which the following is a specification.

My invention relates to electrolytic and flotation processes of treating ore of metals. It has for its more immediate object the treatment of mixed sulfid and oxid ores, especially of copper, although it is not intended to limit it to any particular ore or 15 to any particular combination of minerals in the ore.

It is well known that oxidized ores of copper are not ordinarily amenable to flotation, and that it has been quite a problem to successfully float either oxidized ore, or sulfid 20 ores containing some oxids.

A common method of procedure in flotation is, to add acid to the ore pulp: the acid so added is supposed to help float the mineral, but it is too small in amount to exert any solvent action on the mineral content of the ore, and so far as known, none is claimed. In this process it is intended to add sufficient acid, say, to mixed sulfid and oxid 25 ores of copper, to exert a solvent action on the oxids, and then electrolyze the resulting metal solution in such a way that the electrolytically separated metal is floated, together with the sulfid minerals.

In describing the process more in detail, it may be assumed that the ore under treatment is a mixed sulfid and oxid ore of copper, which is quite common, and which occurs in large deposits in the western part of 30 the United States. The sulfid mineral is usually in the form of chalcocite and chalcopyrite, and the oxid mineral usually in the form of malachite, azurite, and melanite. All the oxid and carbonate ores of 35 copper are easily attacked by all mineral acids. Sulfuric acid, being the most common, will be supposed as being used in the present description.

The ore, usually finely pulverized, is 40 treated with a dilute solution of sulfuric acid. This attacks the oxids, and the copper goes into solution as the sulfate. The acid pulp, in which the sulfids are practically unaffected and the oxids partially or 45 totally converted into the sulfate, is agitated with flotation oils, and the mixture in-

duced into an electrolytic cell in which it can be subjected to electrolysis and flotation. The gas generated by the electrolysis will float the sulfids as usual, and, by using a 60 high current density in the electrolysis, a spongy, non-adherent copper is deposited on the cathodes which is floated, with the sulfids, as rapidly as detached.

In the electrolytic action, under the conditions, the copper will be loosely deposited which is easily detached, acid will be regenerated which will immediately dissolve more copper, ferric salts are formed which are immediately reduced by the action of 70 the minerals in the pulp, and gases such as oxygen and hydrogen are liberated which will float, or materially assist in the flotation of, both the mineral and the metal.

Sponge copper, deposited with a high current density, may float without the assistance of ordinary flotation agents. This is probably due to occluded hydrogen. It is easily floated with the assistance of flotation agents.

While any suitable apparatus may be used, an apparatus, such as shown in diagrammatic section in the accompanying drawing, will be found convenient for carrying out the process.

In the drawing, 1 is a flotation tank containing electrodes 2 and 3, for electrolyzing the ore pulp. Suspended vertically within the tank is a shaft 4, at the upper end of which is attached a pulp distributor 6, and 80 at the lower end an agitator 5. The shaft is rotated by the motor 7. 10 is a thickener, or separator, for separating the liquid from the solids after treatment. 13 is a pump to elevate the liquid from the overflow launder 95 12 to the agitating tank 15. 17 is another thickener, for the finely ground ore pulp, by means of which the water used in grinding is separated from the solids, and the water returned to the grinding mill 19, while 100 the thickened solids flow into tank 15 for acid treatment and mixing of the flotation agent.

In operating the process, the thickened pulp from the mill 19, is flowed into tank 15, 105 where it is treated with acid and oil, so that much of the soluble copper is brought into solution and the pulp mixed with the flotation agent. The pulp then flows into the combined flotation and electrolytic cell 1, 110 distributed by the distributor 6. The electric current in the cell, which is preferably

of a high current density, loosely deposits the copper on the cathodes, while oxygen is liberated at the anodes. Sulfuric acid and ferric sulfate are also produced. Hydrogen 5 may also be liberated at the cathodes. The liberated gases float the sulfid minerals, as also the sponge copper deposited on the cathodes, as rapidly as it becomes detached. The acid and ferric salts regenerated in the 10 pulp dissolve more copper, which is in turn deposited. The deleterious action of the ferric salts, so highly injurious in ordinary electrolysis of impure copper solutions, is overcome by both the high current density 15 and by the oxid and sulfid minerals in the pulp. The stirrer 5, acts to distribute the released gases of electrolysis and give them uniformity of action, and to loosen the deposited copper from the cathodes. It also 20 serves to distribute extraneously introduced gases through the pipe 24, if such gases are desired.

The pulp, now having both the combined and elemental copper largely removed by 25 flotation and electrolysis, is collected in the bottom of the flotation and electrolytic tank, and through the outlet 9, flows with the regenerated acid, into the separator 10, where the regenerated acid solution, containing 30 also usually some copper in solution, is separated from the gangue. The regenerated acid solution, overflowing from the separator 10 into the launder 12, is elevated by means of the pump 13 and pipe line 14, into the tank 15, where it is mixed with fresh pulp from the mill, and the cycle repeated, and thus the process goes on indefinitely. The gangue, separated from most of the liquid used in the electrolysis and flotation, 35 flows out of the separator 10, by the outlet 11, over a gravity concentrator 22, where any of the mineral or electrolytically deposited metal which was too heavy to float, is separated from the gangue by gravity concentration, by any of the well known devices. The small amount of copper sulfate which 40 escaped electrolysis and recovery in the separator 10, may be chemically precipitated if found worth while. The flotation concentrate in the cell 1, overflows into the launder 45 21, and is removed as desired.

It is usually desirable to crush wet: the ore may be crushed in the usual way with the usual amount of water, and then most of 50 the water removed from the solids in the thickener 17, and returned to the mill 19 to pass through another cycle, while the thickened pulp flows into the agitating tank 15 for treatment.

60 The pulp, treated with a flotation agent and a solvent for the copper in tank 15, is distributed over the electrodes in the cell 1, and passes in a downward stream between the electrodes against the current of ascending 65 gases liberated by the electrolytic action,

and in this way, both the mineral and electrolytic metal may be effectively floated. The electrolytic gases, liberated in the pulp, are very effective in flotation, and the agitation of the electrolyte serves to distribute the intensely fine bubbles uniformly through the pulp. The pulp, in passing between the electrodes, comes in contact with the gases at their highest efficiency. Under the action of this process, not much gas is required. 70 75

It is advisable to retain as much of the solution from the separator 10, as possible, in the circuit, for, this solution not only acts as a solvent for the copper, but also as a conductor of the electric current in the elec- 80 85

To the finely ground ore, in the agitator 15, will usually be added enough water and regenerated acid solution to make an easy flowing pulp—much the same as in ordinary 85 flotation work; that is to say, an amount of water equal to about four to six times the weight of the ore. It is preferred to have the solution of the copper, in the agitator 15, go on continuously, and the rate of flow arranged so that about one-fourth of the copper is brought into solution before entering the electrolyzer 1, so that the remainder of the soluble copper can be acted upon by the acid and ferric salts regenerated by the 90 95 electrolytic action. The time of treatment will depend almost entirely upon the nature of the ore and the strength of the acid. Usually, one hour will be sufficient time for acid treatment in the agitator 15, with a five 100 per cent. acid solution. The strength of the acid will depend largely on the amount of soluble copper in the ore, and will usually vary from two to five per cent. Fresh acid may be added from time to time from the 105 acid storage tank 25, as desired. The flotation agent may be added to the agitator 15, from the flotation agent tank 26, or, added afterward to the stream of pulp flowing from the agitator to the electrolyzer. The 110 nature and the amount of flotation agent used, will depend on the nature of the ore, and will have to be determined much the same as in ordinary flotation work. It will usually vary from one-fourth to several per 115 cent. of the weight of the dry ore.

The E. M. F. required will depend mostly on the amount of copper in the solution, the acidity of the solution, its temperature, and very largely on the current density. The 120 current density will usually vary from fifty to one hundred amperes per square foot; with such current densities the E. M. F. required will usually vary from three to five volts. The distance between the electrodes 125 is about the same as in other copper deposition; that is to say, it will vary from one inch to two inches.

The relative amounts of oxid and sulfid minerals will depend, practically, entirely 130

on the product from the mine. The limits will be determined mostly by economic considerations. If the ore is high in oxid minerals and low in sulfids, or, if the ore is composed entirely of oxid minerals, it would probably be better to filter the solutions before electrolyzing, as in ordinary solvent processes: if, however, filtering is difficult, and the purity of the deposited copper is material, there still might be an advantage in using the present method. Ordinarily, it will find its best application in ores containing most of the values in the form of sulfids, and not sufficient oxids to warrant a separate solvent process.

A little experimenting will be necessary for each individual case, to deposit the copper in a non-adherent form on the cathode, so that the copper, as it becomes detached, can be floated from the liquid. In this way the cathodes never need stripping, or removing, but are practically permanent until worn out. On the other hand, the copper so deposited and recovered, is very impure and needs additional refining, as compared with the pure electrolytic metal obtainable by the regular electrolytic solvent processes.

I claim:

1. A metallurgical process which consists in treating mixed sulfid and oxid ores of copper with a solvent for the oxidized copper, applying a flotation agent to the ore pulp, electrolyzing the ore pulp at a current density sufficiently high to give a loose deposit of copper, and floating the metallic copper produced by the electrolysis and the sulfid mineral with gases liberated by the electrolytic action.

2. A process which consists in treating mixed sulfid and oxid ores of copper with a solvent for the oxidized copper, applying a flotation agent to the ore pulp, electrolyzing the ore pulp at a current density sufficiently high to give a loose deposit of copper, and floating the metallic copper and the sulfid mineral from an electrolyzed pulp.

3. A metallurgical process which consists in treating ores of metals with a solvent for the metals, electrolyzing the resulting metal solutions in the presence of the gangue to deposit the metal loosely upon the cathode and capable of being floated by the addition of flotation agents, and recovering the electrolytically loosely deposited metal from the liquid by flotation.

4. A metallurgical process which consists in treating ores of metals with a solvent for the metals, electrolyzing the resulting metal solution to deposit the metal loosely upon the cathode and capable of being floated by flotation agents, and recovering the loosely electrolytically deposited metal from the liquid by flotation.

5. A metallurgical process which consists in treating mixed sulfid and oxid ores of metals with a solvent for the metals, applying a flotation agent to the ore pulp, electrolyzing the pulp, and floating the resulting electrolytic metal with the sulfid mineral.

6. A metallurgical process which consists in treating mixed sulfid and oxid ores of metals with a solvent for the metals, electrolyzing the resulting metal solution to deposit the metal upon the cathode in a form capable of being detached during the electrolysis and capable of being floated by the addition of flotation agents, and recovering the electrolytically deposited metal with the sulfid mineral contained in the ore by flotation.

7. A metallurgical process which consists in treating ores of metals with solvent for the metals, electrolyzing the resulting metal solution with a current density sufficiently high to give a spongy deposit and capable of detaching itself from the cathode and capable of being floated on the addition of flotation agents, and recovering the metal so deposited by flotation.

8. A metallurgical process which consists in mixing finely ground ores of metals with a solvent for the metals and with a flotation agent, electrolyzing the ore pulp, agitating the pulp, and passing the stream of pulp against the ascending gases liberated by the electrolytic action.

9. A metallurgical process which consists in subjecting ores of metals to the action of an electric current in the presence of an acid solution to convert the metal constituents of the ore into the form of sponge metal capable of being floated on the addition of suitable flotation agents, and recovering the resulting electrolytically produced sponge metal from the liquid by flotation.

WILLIAM E. GREENAWALT.

Witnesses:

MARY H. BROOKS,  
IRMA GREENAWALT.